

Jan. 19, 1932.

W. H. RAMAGE

1,841,914

INGOT MOLD

Filed Sept. 1, 1926



INVENTOR  
*William Haig Ramage*  
BY  
*George Ramage*  
his ATTORNEY

## UNITED STATES PATENT OFFICE

WILLIAM HAIG RAMAGE, OF GIRARD, OHIO, ASSIGNOR TO VALLEY MOULD AND IRON CORPORATION, OF HUBBARD, OHIO, A CORPORATION OF NEW YORK

## INGOT MOLD

Application filed September 1, 1926. Serial No. 132,923.

This application relates to metallurgy and more especially to ingot molds, stools, and the like.

That portion of an iron ingot mold or stool which comes into contact with or is adjacent to the molten metal, such as molten steel, when the ingot mold is in use becomes very highly heated, and cools down as the molten steel, comprising the ingot, freezes. This portion of the ingot mold wall or stool is subjected to enormous strains, because the thick metal wall of the iron ingot mold or stool is relatively cool when the steel is first poured in and is quickly raised to a high temperature on the matrix side of the wall, while the outer side of the wall is relatively cool until sufficient time has elapsed to permit the heat to travel through the ingot mold wall. The repeated heating and cooling of the ingot mold by repeated use in casting ingots, subjects the ingot mold to wear which sooner or later destroys the usefulness of the ingot mold. The cost of ingot mold replacement is necessarily an element which enters into the final cost of the steel produced. It therefore follows that the longer the life of the ingot mold can be prolonged before the ingot mold is worn out, the more economical is the production of ingots from such an ingot mold.

One of the factors entering into the destruction of the ingot mold by use is the formation of what are termed in the art "fire-cracks." These cracks start at the matrix surface and gradually deepen and widen as the ingot mold is used. Fire-cracks usually start where an edge of a flake of graphitic carbon extends to the matrix surface of the ingot mold. These cracks may cause chunks or pieces of the matrix side wall to spall off, thus producing a roughened surface which ruins the ingot mold. Furthermore, the fire-cracking action increases the erosive effect of a hot stream of steel where such stream strikes on the ingot mold or stool. The action of erosion is also accelerated or increased by a matrix wall of open grained cast iron, even before serious fire cracking begins to occur. Unfortunately, the kind of metal which is best suited for resisting the

thermal strains set up by repeated heating and cooling of the ingot mold when in use has normally the qualities which are conducive to fire cracking. Therefore, an ingot mold having a matrix wall of open grained metal has a relatively short life.

The present invention overcomes the difficulties heretofore encountered in ingot molds, as above pointed out, by providing an ingot mold construction in which the surface comprising the matrix wall of the ingot mold or stool, and the metal adjacent thereto, is impregnated with metals or metallic substances which close the grain of the cast iron in the side wall adjacent the matrix surface of the ingot mold or stool. Preferably, the materials used for this purpose are of such character as to combine with the carbon in the molten iron when the ingot mold is being cast to form carbides and to cause such graphitic carbon as remains in this part of the ingot mold wall to tend to assume nodular or spheroidal forms instead of comprising graphitic carbon in flake form such as is usually found in open grained metal.

The preferred manner or method of obtaining the desired results may be brought about by applying powdered or pulverized commercial ferro-chrome preferably though not necessarily in a dry form to the matrix portions of the casting molds in which the ingot mold and stool are to be cast.

The matrix portion of the ingot mold is determined by the core of the casting set-up, and the powdered or pulverized ferro-chrome may be applied to the core by any suitable vehicle which will cause this material to adhere to the substantially vertical faces of the core. One convenient vehicle for this purpose comprises blacking which is commonly used on cores for casting ingot molds. Experiments have demonstrated that a satisfactory result is obtained by using ferro-chrome powdered or pulverized to such fineness as to pass a forty mesh screen. Good results have also been obtained by the use of both finer and coarser pulverized ferro-chrome, and by mixtures of fine and coarse powders thereof.

The results are improved by the addition

of substances which give an exothermic reaction. Such a substance which produces this reaction satisfactorily for the present purposes is powdered aluminum mixed with 5 any suitable oxide in proper proportions well known in the art. The aluminum is also beneficial for its physical effect in facilitating troweling or smoothing the ferro-chrome where it is applied in dry powdered form, 10 as is the preferred way of applying it, to surfaces of the casting mold which are horizontal or of such inclination as to permit this method of application.

The following mixtures have produced 15 very satisfactory results, and are given by way of examples of mixtures for carrying out the present invention.

*Mixture "A"—Chrome coating*

|                                    | Per cent<br>by weight |
|------------------------------------|-----------------------|
| Ferro-chrome (69.9% Cr content)    | 92.16                 |
| Anhydrous borax ( $Na_2B_4O_7$ )   | 0.95                  |
| Chrome ore (55% $Cr_2O_3$ content) | 4.59                  |
| Aluminum                           | 2.30                  |

*Mixture "B"—Chrome coating*

|                                    | Per cent<br>by weight |
|------------------------------------|-----------------------|
| Ferro-chrome (69.9% Cr content)    | 85.43                 |
| Anhydrous borax ( $Na_2B_4O_7$ )   | 0.86                  |
| Chrome ore (55% $Cr_2O_3$ content) | 7.28                  |
| Aluminum                           | 3.79                  |
| Magnesium                          | 2.64                  |

*Mixture "C"—Chrome coating*

|                                    | Per cent<br>by weight |
|------------------------------------|-----------------------|
| Ferro-chrome (69.9% Cr content)    | 89.19                 |
| Anhydrous borax ( $Na_2B_4O_7$ )   | 0.90                  |
| Chrome ore (55% $Cr_2O_3$ content) | 6.19                  |
| Aluminum                           | 3.49                  |
| Magnesium                          | 0.23                  |

*Mixture "D"—Chrome coating*

|                                            | Per cent<br>by weight |
|--------------------------------------------|-----------------------|
| Ferro-chrome (69.9% Cr content)            | 83.0                  |
| Magnesium (C. P.)                          | 1.0                   |
| Chrome ore (40% Cr content)                | 6.0                   |
| Aluminum (C. P.)                           | 10.0                  |
| (This mixture has molten resin as a flux.) |                       |

*Mixture "E"—chrome-nickel coating—Dry powder*

|                                    | Per cent<br>by weight |
|------------------------------------|-----------------------|
| Ferro-chrome (69.9% Cr content)    | 14.63                 |
| Nickel (96.5% Ni content)          | 73.30                 |
| Anhydrous borax ( $Na_2B_4O_7$ )   | 0.99                  |
| Chrome ore (55% $Cr_2O_3$ content) | 6.99                  |
| Aluminum                           | 2.69                  |
| Magnesium                          | 1.40                  |

*Mixture "F"—chrome-manganese coating—Dry powder*

|                                    | Per cent<br>by weight |
|------------------------------------|-----------------------|
| Ferro-chrome (69.9% Cr content)    | 61.42                 |
| Ferro-manganese (80% manganese)    | 30.67                 |
| Anhydrous borax ( $Na_2B_4O_7$ )   | 0.93                  |
| Chrome ore (55% $Cr_2O_3$ content) | 3.59                  |
| Aluminum                           | 2.39                  |
| Magnesium                          | 1.00                  |

*Mixture "G"—chrome-titanium coating—Dry powder*

|                                    | Per cent<br>by weight |
|------------------------------------|-----------------------|
| Ferro-chrome (69.9% Cr content)    | 63.0                  |
| Ferrocarbontitanium                | 21.2                  |
| Anhydrous borax ( $Na_2B_4O_7$ )   | 0.8                   |
| Chrome ore (55% $Cr_2O_3$ content) | 10.0                  |
| Aluminum (C. P.)                   | 4.0                   |
| Magnesium (C. P.)                  | 1.0                   |

*APPLICATION: WITH TROWEL*

*60 Mixture "H"—chrome-nickel coating (with anhydrous borax)*

|                                      | Per cent<br>by weight |
|--------------------------------------|-----------------------|
| Ferro-chrome (69.9% Cr content)      | 12.4                  |
| Nickel (96.5% Ni content)            | 61.6                  |
| Anhydrous borax ( $Na_2B_4O_7$ )     | 0.7                   |
| Chrome ore (55.0% $Cr_2O_3$ content) | 6.0                   |
| Aluminum (C. P.)                     | 4.8                   |

|                                                                   |      |
|-------------------------------------------------------------------|------|
| Magnesium (C. P.)                                                 | 1.0  |
| Linseed oil (Sp. G. 0.93)                                         | 13.5 |
| <i>Mixture "I"—chrome-titanium coating (with anhydrous borax)</i> |      |
| Per cent<br>by weight                                             |      |
| Ferro-chrome (69.9% Cr content)                                   | 51.6 |
| Ferrocarbontitanium                                               | 17.2 |
| Anhydrous borax ( $Na_2B_4O_7$ )                                  | 0.7  |
| Chrome ore (55.0% $Cr_2O_3$ content)                              | 11.1 |
| Aluminum (C. P.)                                                  | 4.6  |
| Magnesium (C. P.)                                                 | 1.3  |
| Linseed oil (Sp. G. 0.93)                                         | 13.5 |

These mixtures may be laid on as a coating in varying depths. Satisfactory results have been obtained where the amounts have varied from nine-tenths of a gram per square inch surface covered to three grams per square inch.

Ingot molds cast according to the present invention may be of any shape or type and the grain closing material need be applied only to that part of the set-up which forms the matrix of the ingot mold or stool. The grain closing material appears to soak into or to be absorbed by the molten iron in such manner as to form a compound and where a chromium compound or metallic chromium is used, it appears to form chromium carbide and also a double carbide of chromium and iron, the highest percentage of which is adjacent the treated surface of the cast iron and lesser amounts are to be found at considerable depths in the cast iron. In other words, the process of the present invention forms an admixture of iron and a chromium compound which soaks into the iron and closes the grain of the iron without leaving a coating of metallic chromium on the surface. There is no distinct line of demarcation between the chromium compound and the cast iron but on the contrary, there is a thorough comingling of these materials which decreases in richness of the chromium compound from the surface until all trace of this compound disappears at a depth varying from the surface skin to one-half an inch, dependent on the amount of chromium compound used and the temperature and condition of the molten iron. The greater amount of the carbon adjacent the surface treated appears to be in the form of combined double carbide of iron and chromium and such graphitic carbon as exists appears to be in the form of nodules or spheroids and there does not appear to be any pure chromium present in the finished article.

While chromium compounds have been referred to as the preferred substances, I have found that other ferro alloys will satisfactorily close the grain of the cast iron ingot molds; and as an example of other alloys contemplated by the present invention are ferro manganese; powdered or pulverized washed metal; powdered or pulverized white iron; and the ferro alloys of tungsten, molybdenum, nickel, titanium and other metals of these characters.

The figure of the drawing illustrates in a

conventional way a vertical section through an ingot mold and stool according to the present invention in which the body 1 of the ingot mold and the body 2 of the stool are of ordinary cast iron. The matrix faces 4 of the ingot mold and the matrix faces 5 of the stool are impregnated with a grain closing substance such as ferro-chrome or other ferro alloys above referred to produce fine 10 close grained dense metal adjacent the matrix side wall and which blends into the softer and more open grained metal adjacent the outer side of the walls 6 of the mold and the outer side of the wall 7 of the stool.

15 Having thus described my invention, what I claim is:—

1. An article of manufacture comprising a cast iron ingot mold having a dense close tough matrix side wall comprising an alloy 20 of iron adapted to resist fire cracking and supported by open grained metal.
2. As an article of manufacture, a cast iron ingot mold with the metal adjacent a portion of the matrix surface comprising an 25 alloy of iron having a structure of fine grain crystallization adjacent the matrix surface and gradually blending into a more open crystalline structure comprising cast iron.

WILLIAM HAIG RAMAGE.

20

25

40

45

.50

55

60

65